

Patented Aug. 7, 1945

2,381,854

# UNITED STATES PATENT OFFICE

2,381,854

## SULPHIDES OF ALKYLATED ARYL, OXY-ORGANIC CARBOXYLIC ACIDS

Orland M. Reiff, Woodbury, N. J., assignor to Socony-Vacuum Oil Company, Incorporated, a corporation of New York

No Drawing. Application December 17, 1942,  
Serial No. 469,361

12 Claims. (Cl. 260—516)

This invention has to do with new chemical compounds or reaction products which may be generally designated as the sulphides of alkyl-substituted aryl ether acids or as the sulphides of alkylated aroxy organic carboxylic acids. Although the invention is broadly concerned with chemical compounds or compositions coming within the above-designated general classification, it contemplates as a preferred group coming within such general classification those compounds or condensation products which are soluble or miscible with mineral oil.

My invention is predicated upon the discovery that the oil-miscible compounds or condensation products contemplated herein when blended with a viscous mineral oil fraction such as a hydrocarbon lubricating oil, will improve various properties of the oil. For example, I have found that the compounds or reaction products contemplated herein will inhibit oxidation of the oil, thereby retarding the formation of sludge and acidic products. They also have a peptizing action on such sludge as may be present or as may eventually be formed. Thus, any one of these preferred oil-miscible compounds or condensation products may, for example, be used in internal combustion engine lubricants to retard or prevent the sticking of piston rings, the clogging of piston ring slots, the corrosion of bearings and other parts susceptible to attack by acidic products of oxidation in the oil, and through a proper choice of metal substituent (lead, copper, tin or zinc, for example) the load-carrying ability or lubricity of the oil may be improved.

The alkyl substituents on the aryl nuclei of the compounds or condensation products contemplated herein act to impart oil-miscibility to the product and for the preferred general class of oil miscible compounds these alkyl substituents preferably contain at least twenty carbon atoms. This preferred sub-group of compounds having the so-called "heavy alkyl" groups of at least twenty carbon atoms (such as derived, for example, from a Friedel-Crafts condensation with chlorinated paraffin wax) act to improve the oil in the same respects noted above, and, in addition, they improve the viscosity index and pour point of the oil. A petroleum wax such as paraffin wax constitutes a preferred source for these

so-called heavy alkyl substituents of the latter type and for that reason the preferred multi-functional compounds may be hereinafter designated as "wax"-substituted. It is to be understood, however, that the term "wax" as used in this regard is not restricted to substituent groups derived from petroleum wax but is intended to include substituent groups derived from any aliphatic hydrocarbon or mixture thereof or any 10 predominantly aliphatic material which is in character or constituents similar to the constituents of petroleum wax.

It is to be understood that the present invention is not concerned with mineral oil compositions, such compositions forming the subject matter of my copending application Serial No. 330,693, filed April 20, 1940, now Patent 2,326,496 issued August 10, 1943, of which the present application is a continuation-in-part and to which 20 reference is made for further details in the composition of these compounds or reaction products.

It is also to be understood that the present invention is not confined to the oil-miscible or oil-soluble compounds and that the use of the 25 preferred oil-miscible compounds is not confined to the improvement of mineral oils, since this whole class of new materials is possessed of valuable properties irrespective of oil-miscibility. For example, the compounds or condensation 30 products contemplated herein may be used as intermediates in the production of resins, resin-like materials, rubber substitutes, etc. Certain of the compounds or compositions are possessed of valuable pharmaceutical, insecticidal, or similar 35 properties. Numerous other uses and applications of the compounds or condensation products contemplated herein will be readily apparent to those skilled in the art from the following description of their compositions and a typical 40 method for synthesizing them.

In the aforesaid copending application, which is directed to mineral oil compositions having incorporated therein the compounds or compositions of the present invention, I have distinguished over the chemical compounds or compositions described in Patent 2,198,293, in which I 45 am a co-inventor. Briefly, the compounds or compositions of said patent are alkyl-substituted aryl ether acids; whereas, the compounds or compositions of the present invention are sul-

phides, selenides or tellurides of alkyl-substituted aryl ether acids wherein at least two of said aryl ether acid groups are interconnected by at least one atom of sulphur, selenium or tellurium. Thus, a typical compound or condensation product of the type contemplated herein may be represented by the general formula:



wherein Y represents an element selected from the group consisting of sulphur, selenium and tellurium;  $n$  represents a whole number from one to four;  $\cdot O \cdot Z \cdot COOH$  represents an ether carboxylic acid group (or, oxy-organic carboxylic acid group) in which Z represents an aliphatic, alicyclic or aromatic group; R and R' represent aliphatic hydrocarbon groups containing at least twenty carbon atoms; and x represents a whole number from one to four. It will be noted that this compound is a condensation product of an alkyl-substituted aryl ether acid in which at least one alkyl group (R) is attached to an aryl nucleus and in which an ether acid group is attached to the aryl nucleus through the ether oxygen atom.

It is to be understood, of course, that the aryl nucleus (disclosed in the general formula above as a substituted phenyl group) may be either mono- or poly-cyclic; also that it may carry other substituents, such as ester, keto, alkoxy, alkyl sulphide, aryl sulphide, halogen, hydroxy, amino, nitro, etc., as more fully disclosed in application Serial No. 330,693, of which this is a continuation-in-part. It will be apparent that when the aryl nucleus is poly-cyclic, x may be greater than 4 inasmuch as there are a greater number of replaceable hydrogen atoms than in a phenyl group.

As indicated above, Z may be an aromatic nucleus, and in that event, this aryl nucleus may have R and R' substituents, and also the various substituents referred to above, the condensation with the linkage  $(Y)_n$  may take place between the aryl nucleus or nuclei of such Z group. The foregoing general formula is intended to include such modified derivatives. When Z is aliphatic, certain of the various substituents (exclusive of those of strictly aromatic origin) referred to above may be present therein.

It is to be understood that the term "sulphide," as used herein, is inclusive of the monosulphides, disulphides, trisulphides, tetrasulphides, etc.; that is, it includes both monosulphides and polysulphides and is also inclusive of such polymers and related complex derivatives as may be formed by the procedures described hereinafter. It is to be further understood that the terms: "selenides" and "tellurides" have similar connotations.

As the sulphur derivatives or sulphides of the alkylated aryl ether acids are the preferred class of condensation products contemplated herein, the invention will be specifically described in connection with these derivatives, although, as aforesaid, the selenide and telluride derivatives are contemplated as coming within the scope of the broad inventive concept.

Several general procedures for synthesizing the sulphides of alkylated aryl ether acids may be employed. An alkylated aryl ether acid may be reacted with a sulphur halide, or an alkali metal carboxylate of an alkylated aryl ether acid may be reacted with a sulphur halide. The sulphides

obtained by the latter method are of lighter color than those obtained by the first method and for this reason, the latter method is preferred. Still another desirable procedure consists in conversion of a wax-phenol or wax-alkali phenate to the wax-hydroxy aryl sulphide, followed by introduction of the ether acid group; however, when Z is aromatic, the previously mentioned procedures are preferred.

- 10 In the event sulphur dichloride is used in the foregoing procedures, the condensation products will be monosulphides ( $n=1$  in general Formula I) or polymers thereof; if sulphur monochloride is used, the condensation products will be disulphides ( $n=2$  in general Formula I) or polymers thereof; and if a mixture of sulphur halides is used, the condensation products will be a mixture of sulphides. Monosulphide condensation products are obtained when elementary sulphur is used 20 in place of a sulphur dihalide, but this is not considered the most desirable procedure. Sulphides of higher sulphur content can be formed by reacting a condensation product having the disulphide linkage with elementary sulphur or with an alkali polysulphide or with an alkyl tetrasulphide. Such higher sulphur derivatives may also be obtained by first reducing the disulphide to form the corresponding thiophenol or aryl mercaptan of the alkylated aryl ether acid and then reacting the latter with sulphur dichloride (to form the tri-sulphide) or with sulphur monochloride (to form the tetrasulphide).

30 The alkylated aryl ether acids and their alkali metal salts used in preparing the sulphides may be obtained in various ways. The details in desirable procedures for preparing the alkylated aryl ether acids are described in Patent 2,198,293 referred to above. A typical procedure for preparing the alkali carboxylates and the corresponding alkylated aryl ether acids is described hereinafter.

40 Examples of halogenated organic carboxylic acids which may be used (as their alkali metal salts) in the formation of aryl ether acid derivatives are the halogenated monobasic aliphatic acids such as acetic, butyric, octoic, palmitic, stearic, naphthenic, etc.; polybasic acids such as maleic, succinic, adipic, etc.; and aromatic acids such as benzoic, phthalic, cinnamic, furoic, etc. Both aliphatic and aromatic acids may also carry substituents, such, for example, as keto, nitro, 50 amino, hydroxy groups and the like.

55 The alkylation of the aromatic compound may be carried out in various ways. A preferred procedure is to subject a hydroxyaromatic compound to a Friedel-Crafts condensation reaction with a halogenated aliphatic hydrocarbon, which, for obtaining the preferred multi-functional addition agents, should be an aliphatic hydrocarbon containing at least twenty carbon atoms or a mixture of aliphatic hydrocarbons predominantly comprised of compounds having at least twenty carbon atoms. This alkylation may also be carried out with unsaturated hydrocarbons or aliphatic alcohols, using sulphuric acid or anhydrous aluminium chloride as a catalyst. In alkylating phenols with high molecular weight alcohols, however, it is preferred to convert the alcohol to the corresponding halide (or polyhalide) and then condense the alkyl halide with the hydroxyaromatic 60 compound by the Friedel-Crafts reaction. For obtaining the preferred multi-functional addition agent with unsaturated hydrocarbons or aliphatic alcohols, they should be high molecular weight compounds containing at least twenty carbon atoms, such, for example, as eicosylene, cerotene,

melene, polymerized isobutylene, etc., and myrcyl alcohol, ceryl alcohol, etc.

The Friedel-Crafts synthesis is preferred for obtaining the alkylated hydroxyaromatic compound, and, as a source of the alkyl substituent, preference is given to mixed high molecular weight hydrocarbons typified by those which characterize the heavier products of petroleum, such as heavy petroleum oils of the lubricant type, petrolatum and crystalline petroleum wax or other compounds which will result in relatively long-chain aliphatic substituents. Special preference is given to petroleum wax (paraffin wax) of melting point not substantially less than about 120° F., which is predominantly comprised of aliphatic hydrocarbons having a molecular weight of at least 250 and containing at least twenty carbon atoms.

Hydroxyaromatic compounds which may be used in the alkylation reaction are mono- and poly-cyclic and mono- or poly-hydric hydroxyaromatic compounds which may or may not be otherwise substituted. Specific examples of such compounds are: phenol, resorcinol, hydroquinone, catechol, cresol, xylanol, hydroxy-diphenyl, benzylphenol, phenyl ethyl phenol, phenol resins, methyl hydroxy-diphenyl, alpha- and beta-naphthol, tolyl naphthol, anthrol and the like, with special preference given to phenol and alpha- and beta-naphthol.

Where it is desired to obtain a compound or condensation product in which the aryl nucleus contains in addition to one or more alkyl groups (R and R') or an ether acid group (-O-Z-COOH), another substituent in addition to or in place of residual hydrogen, it is pointed out that with the exception of substituents such as aralkyl, aryl, alkaryl, halogen, hydroxyl and aroxy, such substituent groups are introduced after alkylation and generally before introduction of the ether acid group. The usual methods for the introduction of these substituents into non-alkylated hydroxyaromatic compounds may be employed in connection with the alkylated or wax-substituted hydroxyaromatic compounds contemplated herein. Methods for the introduction of such substituents will be apparent from methods described in Patent 2,198,293, referred to above.

As aforesaid, the preferred products contemplated herein are those having multi-functional properties wherein the alkyl substituent in the aryl nucleus contains at least twenty carbon atoms. In this preferred class of compounds special preference is given to the condensation products derived from alkyl-substituted hydroxyaromatic compounds in which the alkyl substituent is derived from petroleum wax. The details in a typical procedure for synthesizing these so-called wax-substituted hydroxyaromatic compounds (wax-phenol) are described in my Patent 2,197,833. Briefly, this procedure involves reacting a chlorinated wax, such as chlorinated paraffin wax, with a phenol in the presence of a Friedel-Crafts catalyst at elevated temperature. The chlorinated wax should have a chlorine content of from about 10 per cent to about 16 per cent, and the reaction mixture may contain about three atomic proportions of chlorine (in a chlorwax of 16 per cent chlorine content) to one molecular proportion of phenol. A "wax-phenol" obtained from such a reaction mixture may be designated as wax-phenol (3-16). Parenthetical expressions of the type (A-B) will be used hereinafter in connection with the wax-substituted derivatives to designate: (A) the number of atomic propor-

tions of chlorine in the chlorinated wax reacted with one mol of hydroxyaromatic compound, and (B) the chlorine content of the chlorinated wax. In the above example, A = 3 and B = 16. The same designation will also apply to the sulphides of the wax-aroxy organic carboxylic acids which constitute the ultimate product derived from the wax-phenol.

Illustrative procedures which may be followed in preparing the sulphides of alkyl-substituted aryl ether acids contemplated herein are given in the following examples:

#### EXAMPLE I

##### *Preparation of di(wax-phenoxy acetic acid) disulphide*

###### (a) Reaction mixture:

|                                  |       |       |
|----------------------------------|-------|-------|
| Monochloracetic acid             | grams | 127.5 |
| Ethanol                          | cc    | 100   |
| Sodium hydroxide                 | grams | 54    |
| Wax sodium phenate (3-16)        | do    | 200   |
| Mineral oil S. U. V. of 67 secs. |       |       |
| @ 210° F.                        | do    | 600   |
| Sulphur monochloride             | do    | 19.7  |

###### (b) Procedure:

Wax sodium phenate (3-16) was prepared by reacting wax-phenol (3-16), obtained according to the procedure outlined in my Patent 2,197,833, with sodium butylate at about 300° F. and distilling off the alcohol.

A solution of 127.5 grams of monochloracetic acid in 100 cc. of anhydrous alcohol was converted to sodium chloracetate by adding thereto a standard alcohol solution of sodium hydroxide, maintaining the reaction temperature at about 100° F. This sodium chloracetate mixture was then added to a solution of 200 grams of the wax sodium phenate (3-16) in 600 grams of the mineral oil and the mixture was stirred at 150° F. during a two-hour period to form the wax-substituted phenoxy sodium acetate. The temperature was then lowered to about 100° F. and the mixture was sulphurized by adding, with rapid stirring, 19.7 grams of sulphur monochloride at a rate sufficiently slow to avoid appreciable rise in temperature of the mixture by the heat of reaction developed. The mixture was then stirred at this temperature for about one hour to complete the sulphurization, followed by distilling off the alcohol and water-washing the mixture until the aqueous extract was neutral. All traces of alcohol and water were then removed by steam-treating the mixture at about 300° F. to obtain the finished product, which was approximately a one-fourth blend in mineral oil.

The pure di(wax-phenoxy acetic acid) disulphide is obtained in the free condition (rather than in a mineral oil blend) by using a light boiling distillate such as Stoddard's Solvent as the diluent in place of mineral oil, and following the foregoing procedure and finally distilling off said light boiling distillate.

#### EXAMPLE II

##### *Preparation of di(wax-phenoxy benzoic acid) disulphide*

###### (a) Reaction mixture:

|                                               |       |     |
|-----------------------------------------------|-------|-----|
| Brom sodium benzoate                          | grams | 29  |
| Wax sodium phenate                            | do    | 100 |
| Mineral oil of S. U. V. of 67 secs. @ 210° F. | do    | 300 |
| Sulphur monochloride                          | do    | 9.8 |
| Chlorbenzene                                  | cc    | 100 |

## (b) Procedure:

A solution of 100 grams of wax sodium phenate (obtained as in Example I (b)) in 300 grams of the mineral oil was mixed with 29 grams of brom sodium benzoate and stirred at a reaction temperature of about 400° F. during a four-hour period with copper powder as catalyst, to form the disodium salt of (wax-phenoxy benzoic acid). The reaction mixture was then filtered to remove sodium bromide, copper powder, and any unreacted brom sodium benzoate. The filtrate was diluted with 100 cc. of chlorbenzene, and the sulphurization was carried out by adding 9.8 grams of sulphur monochloride at 100° F. at a rate sufficiently slow to avoid appreciable temperature rise by the heat of reaction, and stirring one hour at the temperature to complete the sulphurization, whereby the di(wax-phenoxy benzoic acid) disulphide is formed. The product was purified by water-washing the mixture until the aqueous extract was neutral, followed by distilling off the chlorbenzene diluent to obtain the finished product, which was approximately a one-fourth blend in mineral oil.

As indicated above in Example I (b), the pure di(wax-phenoxy benzoic acid) disulphide is obtained in the free condition by replacing the mineral oil used above as a diluent with a light boiling diluent such as, for example, Stoddard's Solvent, and following the procedure outlined above and finally distilling off said light boiling distillate.

It will be understood that when a mixture of aliphatic hydrocarbon compounds, such as petroleum wax, for example, is used as the source of the alkyl substituents, the resulting composition will be an intimate mixture of compounds or sulphides of alkyl-substituted aryl ether acids, which compounds differ from each other with respect to the nature of the alkyl substituent. In other words, where the alkylation of the aryl nucleus has been effected with a mixture of aliphatic hydrocarbons, the resulting product will likewise be a mixture of compounds differing with respect to the alkyl substituent but having in common the same ether acid group (O-Z-COOH) and the same characterizing aryl nucleus discussed above.

Compounds or condensation products of both the oil-miscible and non-miscible types have been prepared, and of the oil-miscible products which have been tested in mineral oil compositions all have effected improvement in the properties of the oil. The following examples are illustrative of the various oil-miscible sulphides of wax-substituted aryl ether acids which I have prepared and tested to demonstrate their value as addition agents for viscous mineral oils:

Di(wax-phenoxy acetic acid) monosulphide (3-16)  
 Di(wax-phenoxy acetic acid) disulphide (3-16)  
 Di(wax-phenoxy acetic acid) tetrasulphide (3-16)  
 Di(wax-naphthoxy acetic acid) disulphide (3-19)  
 Di(wax-phenoxy butyric acid) disulphide (3-16)  
 Di(wax-phenoxy naphthenic acid) monosulphide (3-16)  
 Di(wax-phenoxy benzoic acid) monosulphide (3-16)  
 Di(wax-phenoxy benzoic acid) trisulphide (3-16)  
 Di(wax-naphthoxy benzoic acid) disulphide (3-19)  
 Di(wax-phenoxy toluic acid) disulphide (2-15)

It is to be understood that although I have described certain preferred procedures for synthesizing the products contemplated by this invention and have listed a number of illustrative com-

pounds or condensation products which are typical thereof, the invention is not limited to the particular procedures or products but includes within its scope such changes and modifications as fairly come within the spirit of the appended claims.

## I claim:

1. As a new composition of matter, a condensation product having the general formula:



15 in which  $n$  represents the number of sulphur atoms and is a whole number from 1 to 4; O-Z-COOH represents an oxy-organic carboxylic acid group in which Z is selected from the group of organic groups consisting of aliphatic, alicyclic and aromatic groups; R and R' represent aliphatic hydrocarbon groups containing at least twenty carbon atoms; and x represents a whole number from 1 to 4.

2. As a new composition of matter, a condensation product having the general formula:



30 in which  $n$  represents the number of sulphur atoms and is a whole number from 1 to 4; O-Z-COOH represents an oxy-aliphatic carboxylic acid group in which Z is an aliphatic group; R and R' represent aliphatic hydrocarbon groups containing at least twenty carbon atoms; and x represents a whole number from 1 to 4.

3. As a new composition of matter, a condensation product having the general formula:



35 in which  $n$  represents the number of sulphur atoms and is a whole number from 1 to 4; O-Z-COOH represents an oxy-aromatic carboxylic acid group in which Z is an aromatic group; R and R' represent aliphatic hydrocarbon groups containing at least twenty carbon atoms; and x represents a whole number from 1 to 4.

4. As a new composition of matter, a condensation product having the general formula:



45 in which  $n$  represents the number of sulphur atoms and is a whole number from 1 to 4; O-Z-COOH represents an oxy-aromatic carboxylic acid group in which Z is an aromatic group; R and R' represent aliphatic hydrocarbon groups containing at least twenty carbon atoms; and x represents a whole number from 1 to 4.

5. As a new composition of matter, a condensation product having the general formula:



in which  $n$  represents the number of sulphur atoms and is a whole number from 1 to 4;  $O\cdot Z\cdot COOH$  represents an oxy-aromatic carboxylic acid group in which  $Z$  is an aromatic group;  $R$  and  $R'$  represent alkyl substituents having at least twenty carbon atoms and derived from paraffin wax; and  $x$  represents a whole number from 1 to 4.

6. As a new composition of matter, a condensation product characterized by at least two aryl nuclei interconnected by at least one atom of sulphur, each of said aryl nuclei being substituted with: (a) at least one alkyl substituent, a carbon atom of which is directly connected to a nuclear carbon atom of one of said aryl nuclei; and (b) at least one oxy-organic carboxylic acid group, the oxygen atom of said oxy-organic carboxylic acid group being directly connected to a nuclear carbon atom of one of said aryl nuclei.

7. As a new composition of matter, a condensation product characterized by at least two aryl nuclei interconnected by at least one atom of sulphur, each of said aryl nuclei being substituted with: (a) at least one alkyl substituent having at least twenty carbon atoms, a carbon atom of which is directly connected to a nuclear carbon atom of one of said aryl nuclei; and (b) at least one oxy-organic carboxylic acid group, the oxygen atom of said oxy-organic carboxylic acid group being directly connected to a nuclear carbon atom of one of said aryl nuclei.

8. As a new composition of matter, a condensation product characterized by at least two aryl nuclei interconnected by at least one atom of sulphur, each of said aryl nuclei being substituted with: (a) at least one alkyl substituent having at least twenty carbon atoms and derived from paraffin wax, a carbon atom of which is directly connected to a nuclear carbon atom of one of said aryl nuclei; and (b) at least one oxy-organic carboxylic acid group, the oxygen atom of said oxy-organic carboxylic acid group being directly connected to a nuclear carbon atom of one of said aryl nuclei.

9. As a new composition of matter, a condensation product having the general formula:



in which  $n$  represents the number of sulphur atoms and is a whole number from 1 to 4;  $O\cdot Z\cdot COOH$  represents an oxy-organic carboxylic acid group in which  $Z$  is selected from the group of organic groups consisting of aliphatic, alicyclic and aromatic groups;  $R$  and  $R'$  represent alkyl substituents having at least twenty carbon atoms and derived from paraffin wax; and  $x$  represents a whole number from 1 to 4.

10. As a new composition of matter, a di(wax-phenyl, oxy-acetic acid) disulphide in which the disulphide group joins the two wax-phenyl groups at nuclear carbon atoms thereof and in which each wax-phenyl group is attached at a nuclear carbon atom to an oxy group which is also attached to an acetic acid group, the said wax groups having at least twenty carbon atoms and derived from paraffin wax.

11. As a new composition of matter, a di(wax-phenyl, oxy-benzoic acid) disulphide in which the disulphide group joins the two wax-phenyl groups at nuclear carbon atoms thereof and in which each wax-phenyl group is attached at a nuclear carbon atom to an oxy group which is also attached to a benzoic acid group, the said wax groups having at least twenty carbon atoms and derived from paraffin wax.

12. As a new composition of matter, an intimate mixture of condensation products characterized by at least two aryl nuclei interconnected by at least one atom of sulphur, each of said aryl nuclei being substituted with: (a) at least one alkyl substituent, a carbon atom of which is directly connected to a nuclear carbon atom of one of said aryl nuclei; and (b) at least one oxy-organic carboxylic acid group, the oxygen atom of said oxy-organic carboxylic acid group being directly connected to a nuclear carbon atom of one of said aryl nuclei; the said condensation products differing from each other with respect to the alkyl substituent, the said alkyl substituents comprising essentially aliphatic hydrocarbon groups having a composition corresponding substantially to the different aliphatic hydrocarbons contained in paraffin wax.

ORLAND M. REIFF.